

June 13, 1967

P. TALMEY ET AL

3,325,297

PROCESSES OF CONTINUOUS CHEMICAL NICKEL PLATING

Filed April 9, 1956



INVENTOR.

Paul Talmey, Gregoire Gutzeit &  
BY Donald E. Metheny.

Smith, Olsen, Baird & Miller

Atty's.

1

3,325,297

## PROCESSES OF CONTINUOUS CHEMICAL NICKEL PLATING

Paul Talmey, Barrington, Ill., and Gregoire Gutzeit, Highland, and Donald E. Metheny, Hammond, Ind., assignors to General American Transportation Corporation, Chicago, Ill., a corporation of New York

Filed Apr. 9, 1956, Ser. No. 576,931  
23 Claims. (Cl. 106—1)

This application is a continuation-in-part of the copending application of Paul Talmey, Gregoire Gutzeit and Donald E. Metheny, Ser. No. 479,040, filed Dec. 31, 1954, now abandoned.

The present invention relates to processes of continuous chemical nickel plating of catalytic materials; and it is the general object of the invention to provide an improved process of the general character of that disclosed in U.S. Patent No. 2,717,218, granted on Sept. 6, 1955 to Paul Talmey and William J. Crehan.

The chemical nickel plating of a catalytic material employing an aqueous bath of the nickel cation hypophosphite anion type is based upon the catalytic reduction of nickel cations to metallic nickel and the corresponding oxidation of hypophosphite anions to phosphite anions with the evolution of hydrogen gas at the catalytic surface. The reactions take place when the body of catalytic material is immersed in the plating bath, and the exterior surface of the body of catalytic material is coated with nickel. The following elements are catalytic for the oxidation of hypophosphite anions and thus may be directly nickel plated: iron, cobalt, nickel, ruthenium, rhodium, palladium, osmium, iridium and platinum. The following elements are examples of materials which may be nickel plated by virtue of an initial displacement deposition of nickel thereon either directly or through a galvanic effect: copper, silver, gold, beryllium, germanium, aluminum, carbon, vanadium, molybdenum, tungsten, chromium, selenium, titanium and uranium. The following elements are examples of non-catalytic materials which ordinarily may not be nickel plated: bismuth, cadmium, tin, lead and zinc. The activity of the catalytic materials varies considerably and the following elements are particularly good catalysts in the chemical nickel plating bath: iron, cobalt, nickel and palladium. The chemical nickel plating process is autocatalytic since both the original surface of the body being plated and the nickel metal that is deposited on the surface thereof are catalytic. As time proceeds, the anions, as contrasted with the cations of the nickel salt that is dissolved in the plating bath, combine with the hydrogen cations to form an acid, which, in turn, lowers the pH of the plating bath.

In the continuous plating process disclosed in the Talmey and Crehan patent, the plating bath is regenerated continuously by the addition thereto of soluble nickel-containing and hypophosphite-containing reagents, as well as an alkalizing reagent for pH control; which regeneration of the plating bath during the plating of the catalytic material maintains not only the desired nickel cation concentration and hypophosphite anion concentration, but also preserves the most advantageous pH of the plating bath to assure a high plating rate. The continuous nickel plating process and system disclosed in this patent involves a plating chamber and a reservoir; and in the arrangement the plating solution is circulated from the reservoir to the plating chamber and back to the reservoir, the plating solution being heated to a relatively high temperature slightly below the boiling point thereof after withdrawal from the reservoir and before introduction into the plating chamber, and the plating solution being cooled to a relatively low temperature well below the boiling point thereof after withdrawal from

2

the plating chamber and before return into the reservoir. Of course, the catalytic body or bodies are plated by immersion in the plating solution in the plating chamber, while the plating solution is regenerated in the reservoir by the addition of the previously mentioned reagents thereto in the reservoir. The catalytic body is subsequently withdrawn from the plating solution in the plating chamber after a time interval corresponding to the thickness of the nickel plating thereon that is desired.

A number of suitable aqueous chemical nickel plating baths of the nickel cation-hypophosphite anion type that may be employed in the continuous nickel plating system of the Talmey and Crehan patent are disclosed in U.S. Patent No. 2,658,841, granted on Nov. 10, 1953, to Gregoire Gutzeit and Abraham Krieg, and in U.S. Patent No. 2,658,842, granted on Nov. 10, 1953, to Gregoire Gutzeit and Ernest J. Ramirez, and in the copending applications of Gregoire Gutzeit, Paul Talmey and Warren G. Lee, Ser. No. 478,492, filed Dec. 29, 1954, now Patent No. 2,935,425, granted May 3, 1960, Ser. No. 479,088, filed Dec. 31, 1954, now Patent No. 2,822,293, granted Feb. 4, 1958 and Ser. No. 569,815, filed Mar. 6, 1956, now Patent No. 2,822,294, granted Feb. 4, 1958. In the continuous plating system, the plating bath disclosed in the Gutzeit, Talmey and Lee applications are preferred, both from the standpoint of economy and of performance, and four typical examples of such aqueous plating baths are as follows:

### BATH I

|                                              |       |                         |              |
|----------------------------------------------|-------|-------------------------|--------------|
| Nickel ions (as nickel sulfate)              | ----- | m.p.l.                  | 0.08         |
| Hypophosphite ions (as sodium hypophosphite) | ----- | m.p.l.                  | 0.230        |
| Lactic acid                                  | ----- | m.p.l.                  | 0.30 to 0.40 |
| Lead ions (stabilizer)                       | ----- | p.p.m. Pb <sup>++</sup> | 1            |

pH adjusted to 4.6 with NaOH.

### BATH II

|                                              |       |                         |              |
|----------------------------------------------|-------|-------------------------|--------------|
| Nickel ions (as nickel sulfate)              | ----- | m.p.l.                  | 0.07 to 0.08 |
| Hypophosphite ions (as sodium hypophosphite) | ----- | m.p.l.                  | 0.225        |
| Lactic acid                                  | ----- | m.p.l.                  | 0.30 to 0.40 |
| Propionic acid                               | ----- | m.p.l.                  | 0.03         |
| Lead ions (stabilizer)                       | ----- | p.p.m. Pb <sup>++</sup> | 1            |

pH adjusted to 4.6 with NaOH.

### BATH III

|                                              |       |                         |       |
|----------------------------------------------|-------|-------------------------|-------|
| Nickel ions (as nickel sulfate)              | ----- | m.p.l.                  | 0.08  |
| Hypophosphite ions (as sodium hypophosphite) | ----- | m.p.l.                  | 0.225 |
| Lactic acid                                  | ----- | m.p.l.                  | 0.20  |
| Succinic acid                                | ----- | m.p.l.                  | 0.06  |
| Lead ions (stabilizer)                       | ----- | p.p.m. Pb <sup>++</sup> | 1     |

pH adjusted to 4.6 with NaOH.

### BATH IV

|                                              |       |                         |       |
|----------------------------------------------|-------|-------------------------|-------|
| Nickel ions (as nickel sulfate)              | ----- | m.p.l.                  | 0.07  |
| Hypophosphite ions (as sodium hypophosphite) | ----- | m.p.l.                  | 0.230 |
| Malic acid                                   | ----- | m.p.l.                  | 0.06  |
| Lactic acid                                  | ----- | m.p.l.                  | 0.20  |
| Succinic acid                                | ----- | m.p.l.                  | 0.20  |
| Lead ions (stabilizer)                       | ----- | p.p.m. Pb <sup>++</sup> | 1     |

pH adjusted to 4.6 with NaOH.

In addition, each of the Baths I, II, III and IV contains a high-temperature stable, chemically inert, wetting agent of any suitable type, and in these baths the function of the organic additives (malic acid, lactic acid, succinic acid and propionic acid) is three-fold, as they act as: (1) buffers; (2) exaltants (plating rate "boosters"); (3) complexing agents (to prevent precipi-

tations of nickel phosphite at high concentrations of  $\text{HPO}_3^{2-}$  ions.

Of these organic additives, lactic acid combines the three effects named, succinic and propionic acids function principally as exaltants, while malic acid functions mainly as a complexing agent.

In the formulation of any one of these plating baths, an aqueous solution is prepared of the ingredients named; the nickel cations may be derived from nickel sulfate, nickel chloride, etc., or various combinations thereof; the hypophosphite anions may be derived from sodium hypophosphite, potassium hypophosphite, etc., or various combinations thereof; the other additives are introduced into the bath normally as the acids, or as the soluble salts thereof, etc.; and the desired pH of the bath is established by the eventual introduction thereto of an acid or a base, as required, sulfuric acid and sodium hydroxide being recommended as a matter of economy and simplicity.

In the compositions of the various plating baths, the terms "cation," "anion" and "ion," as employed, include the total quantity of the corresponding elements that are present in the plating bath, i.e., both the undissociated and dissociated material. In other words 100% dissociation is assumed when the terms noted are used in connection with molar ratios and concentrations in the plating bath.

In the operation of the continuous plating system disclosed in the Talmey and Crehan patent, the whole body of plating solution, as a matter of volume, is continuously circulated from the reservoir to the plating chamber and back to the reservoir to constitute what may be termed a "cycle" of circulation; and continuous regeneration thereof is accomplished in the reservoir by the continuous introduction thereto of the reagents previously mentioned. Now after the whole body of plating solution has been used in production plating in a plurality of cycles of circulation, with the required regeneration thereof, its content in phosphite anions builds-up to a point where even the presence of relatively large quantities of complexing agents (necessarily rather weak complexing agents) cannot prevent the precipitation of nickel phosphite therein. This point is reached when the phosphite concentration attains 0.7 to 1.5 m.p.l., depending on the particular bath composition. The nickel phosphite precipitate in the plating solution forms a suspensoid whose semi-colloidal particles causes roughness of the plating on the catalytic bodies undergoing the plating operation, and also act as nuclei for thermal catalytic decomposition of the whole body of plating solution, i.e., the formation of "black precipitate" therethrough. When this point is reached, the whole body of plating solution may be termed "depleted" and has to be replaced with a freshly prepared body of plating solution in order to continue satisfactory plating of the catalytic bodies in the plating chamber.

A depleted plating bath may have, for instance, the following approximate composition:

|                    | M.p.l.    |
|--------------------|-----------|
| Nickel ions        | 0.07-0.08 |
| Hypophosphite ions | 0.22-0.24 |
| Phosphite ions     | 0.70-1.50 |
| Sulphate ions      | 0.65-0.70 |
| Lactic ions        | 0.20-0.40 |
| Sodium ions, q.s.  |           |

Typical examples of a few depleted plating baths of the type previously described were found to have the following compositions:

#### DEPLETED BATH IA

M.p.l.

|                           |      |
|---------------------------|------|
| Ni ions                   | 0.07 |
| $\text{NaH}_2\text{PO}_2$ | 0.22 |
| $\text{Na}_2\text{HPO}_3$ | 0.80 |
| Lactic acid               | 0.30 |

#### DEPLETED BATH IIA

|                           |      |
|---------------------------|------|
| Ni ions                   | 0.07 |
| $\text{NaH}_2\text{PO}_2$ | 0.22 |
| $\text{Na}_2\text{HPO}_3$ | 0.80 |
| Lactic acid               | 0.30 |
| Propionic acid            | 0.03 |

#### DEPLETED BATH IIIA

|                           |       |
|---------------------------|-------|
| Ni ions                   | 0.084 |
| $\text{NaH}_2\text{PO}_2$ | 0.201 |
| $\text{Na}_2\text{HPO}_3$ | 0.671 |
| Lactic acid               | 0.20  |
| Succinic acid             | 0.06  |

#### DEPLETED BATH IVA

|                           |        |
|---------------------------|--------|
| Ni ions                   | 0.068  |
| $\text{NaH}_2\text{PO}_2$ | 0.225  |
| $\text{Na}_2\text{HPO}_3$ | 0.74   |
| Malic acid                | 0.06   |
| Lactic acid               | 0.2025 |
| Succinic acid             | 0.20   |

#### DEPLETED BATH IVB

|                           |      |
|---------------------------|------|
| Ni ions                   | 0.07 |
| $\text{NaH}_2\text{PO}_2$ | 0.20 |
| $\text{Na}_2\text{HPO}_3$ | 0.86 |
| Malic acid                | 0.06 |
| Lactic acid               | 0.20 |
| Succinic acid             | 0.20 |

While the regeneration of the plating solution in the continuous plating process as disclosed in the Talmey and Crehan patent, and involving the continuous addition thereto of the reagents mentioned, contributes very substantially to economical industrial plating operation, it is apparent that this regeneration of the plating solution does not proceed as far as is desirable in order to achieve maximum economy, since it will be observed from the compositions of the foregoing depleted plating baths that there are substantial values therein that might be further utilized.

Accordingly, it is another object of the invention to provide a continuous chemical nickel plating process of the character described that involves regeneration of the plating baths, not only by the addition thereto of nickel-containing and hypophosphite-containing and alkalizing reagents, but also by the removal therefrom of phosphite ions, whereby depleted plating baths may be restored for further use.

A further object of the invention is to provide an improved process of restoring a depleted chemical nickel plating bath so that it may be employed for further use in the plating of catalytic bodies, which involves not only the removal of phosphite ions therefrom, but also the removal of other ions that have been built-up therein as a consequence of the additions thereto of the reagents named.

A still further object of the invention is to provide an improved process of restoring a depleted chemical nickel plating bath so that it may be employed for further use in the plating of catalytic bodies, which does not introduce any substantial foreign ions thereto and which effects the recovery of the valuable nickel cations, hypophosphite anions and organic additives therein.

The present invention is predicated upon the discovery that a depleted chemical nickel plating bath may be restored for further satisfactory use in a continuous chemical nickel plating system of the character described, by proper treatment of the depleted plating bath to remove therefrom phosphite anions and other ions that have been built-up therein by the addition of the make-up reagents, without the introduction of foreign ions, so that the resulting aqueous solution fundamentally containing nickel cations, hypophosphite anions and organic additives may then be directly restored merely by adding thereto nickel-containing, hypophosphite-containing and acidifying or alkalizing reagents.

Still further features of the invention pertain to the particular arrangement of the steps of the process, whereby the above-outlined and additional operating features thereof are attained.

The invention, both as to its organization and principle of operation, together with further objects and advantages thereof, will best be understood by reference to the following specification taken in connection with the accompanying drawing, in which the single figure is a diagrammatic illustration of a continuous nickel plating system in which the process of the present invention may be carried out.

Referring now to the drawing, the continuous chemical nickel plating system there illustrated, and suitable for the carrying out of the present process, is essentially of the arrangement disclosed in the Talmey and Crehan patent. More particularly, the system fundamentally comprises a first reservoir 11a, a second reservoir 11b, a plating tank or chamber 12, a condenser 13, a primary vacuum flash tank 14, a secondary vacuum flash tank 15, a primary steam jet pump 16, a secondary steam jet pump 17, and a mechanical pump 18. The reservoir 11a includes a baffled storage compartment 19a and a communicating regeneration compartment 20a; while the reservoir 11b includes a baffled storage compartment 19b and a communicating regeneration compartment 20b. In the arrangement, the inlet of the pump 18 selectively communicates with the upper and lower portions of the storage compartments 19a and 19b via respectively associated control valves 21a-22a and 21b-22b; and the outlet of the pump 18 communicates with the upper portion of the condenser 13. The lower portion of the condenser 13 communicates with the upper portion of the plating tank 12; and the lower portion of the plating tank 12 communicates with the upper portion of the primary vacuum flash tank 14. The lower portion of the primary vacuum flash tank 14 communicates with the upper portion of the secondary vacuum flash tank 15; and the lower portion of the secondary vacuum flash tank 15 selectively communicates with the upper portions of the regeneration compartments 20a and 20b via respectively associated control valves 23a and 23b. Also, the upper portion of the primary vacuum flash tank 14 communicates with the primary steam jet pump 16, that is also connected to an associated source of high-pressure steam, not shown; and the discharge from the primary steam jet pump 16 communicates with the upper portion of the condenser 13. Also, the upper portion of the secondary vacuum flash tank 15 communicates with the secondary steam jet pump 17, that is also connected to the associated source of high-pressure steam, not shown; and the discharge from the secondary steam jet pump 17 communicates with the atmosphere. This system contains an aqueous chemical plating solution of the character previously described; whereby a first portion of the plating solution is stored in one of the reservoirs 11a or 11b at a relatively low temperature well below the boiling point thereof and in a relatively concentrated form; while a second portion of the plating solution is held as a bath in the plating tank or chamber 12 at a relatively high temperature slightly below the boiling point thereof and in a relatively dilute form.

In the operation of the system, the plating solution in the storage compartment 19a or 19b may have a temperature of about 150° F.; while the plating solution in the plating tank 12 may have a temperature of about 210° F. The plating solution is circulated from the upper portion of the storage compartment 19a or 19b (depending upon which of the control valves 21a or 21b occupies its open position) by the pump 18 into the upper portion of the condenser 13, wherein it is both heated to the required temperature of about 210° F. and diluted to the required concentration by the discharge from the primary steam jet pump 16. The dilution of the plating solution in the condenser 13 is achieved not only by the introduction of the steam thereinto, but also by the introduction of the water vapor thereinto that is withdrawn

from the upper portion of the primary vacuum flash tank 14 by the primary steam jet pump 16. The plating solution from the condenser 13 is circulated into the plating tank tank 12 and thence into the upper portion of the primary vacuum flash tank 14 and therefrom into the upper portion of the secondary vacuum flash tank 15, and ultimately back into the upper portion of the regeneration compartment 20a or 20b (depending upon which of the control valves 23a or 23b occupies its open position). In the primary vacuum flash tank 14, a vacuum of about 12" Hg is drawn by the primary steam jet pump 16; whereby water vapor is withdrawn from the contained plating solution, as previously noted, so that the plating solution in the primary vacuum flash tank 14 is both concentrated and cooled prior to introduction into the secondary vacuum flash tank 15. In the secondary vacuum flash tank 15, a vacuum of about 22" Hg is drawn by the secondary steam jet pump 17; whereby water vapor is withdrawn from the contained plating solution, so that the plating solution in the secondary vacuum flash tank 15 is both further concentrated and cooled prior to the return thereof to the regeneration compartment 20a or 20b. The plating solution returned into the regeneration compartment 20a or 20b may have a temperature of about 150° F., as previously noted, as a consequence of the tandem cooling effects produced in the primary vacuum flash tank 14 and in the secondary vacuum flash tank 15. Also, the plating solution thus returned to the regeneration compartment 20a or 20b is in the relatively concentrated form, as previously noted, as a consequence of the tandem concentrating effects produced in the primary vacuum flash tank 14 and in the secondary vacuum flash tank 15. Since the discharge of the secondary steam jet pump 17 is to the atmosphere, the water vapor withdrawn from the plating solution in the upper portion of the secondary vacuum flash tank 15 prevents the build-up of water in the circulated plating solution; and preferably, the weight of the steam introduced into the plating solution in the condenser 13 by the primary steam jet pump 16 substantially equals the weight of the water vapor withdrawn therefrom in the secondary vacuum flash tank 15 and discharged to the atmosphere by the secondary steam jet pump 17, thereby maintaining the desired balance of the weight of water supplied to and the weight of water extracted from the circulated plating solution.

The catalytic bodies are immersed in the plating bath in the plating chamber 12, whereby the metallic nickel (actually an alloy of nickel and phosphorous having a composition of about 89% to 97% nickel and 11% to 3% phosphorous by weight) is deposited upon the surfaces thereof; and the bodies are withdrawn from the plating bath when the coatings thereon are of the desired thickness. Incident to the plating of the nickel upon the catalytic bodies, the initial composition of the plating bath is altered by the reduction of the nickel cations and the oxidation of the hypophosphite anions, as previously noted, and the initial pH of the bath is reduced, as previously explained; whereby it is necessary to regenerate the plating solution in the regeneration compartment 20a or 20b by the addition thereto of an alkalinizing reagent to restore the initial pH thereof and of a soluble nickel salt and a soluble hypophosphite to restore the initial composition thereof with respect to nickel cations and hypophosphite anions, the reagents mentioned being supplied into the regeneration compartment 20a or 20b, and being thoroughly dissolved and mixed therewith before circulation back into the communicating storage compartment 19a or 19b.

Further, the system comprises make-up equipment 30 that may include five tanks 31 to 35, inclusive, that selectively communicate with make-up conduits 36 and 37 communicating with the regeneration compartments 20a and 20b. More particularly, the tanks 31 to 35, inclusive, may be selectively connected to the conduit 36 via respective control valves 41 to 45, inclusive, and the

tanks 31 to 35, inclusive, may be selectively connected to the conduit 37 via respective control valves 51 to 55, inclusive. As a matter of convenience, the added alkalinizing reagent may be derived from an aqueous sodium hydroxide stock solution stored in the tank 31, the added nickel reagent may be derived from an aqueous nickel sulfate stock solution stored in the tank 32, the added hypophosphite reagent may be derived from an aqueous sodium hypophosphite stock solution stored in the tank 33, water may be stored in the tank 34, and an aqueous sulfuric acid stock solution may be stored in the tank 35. It will be understood that the valves 41, 42, 43 and 44 are appropriately manipulated in order to bring about the required addition of the reagents from the tanks 31, 32, 33 and 34 into the regeneration compartment 20a, while the valves 51, 52, 53 and 54 are appropriately manipulated in order to bring about the required addition of the reagents from the tanks 31, 32, 33 and 34 into the regeneration compartment 20b.

Finally, the system comprises apparatus 60 that is employed, as explained more fully hereinafter, for the removal of phosphite and other ions, the inlet to the apparatus 60 being selectively connected to the lower portion of the secondary vacuum flash tank 15 via an associated control valve 61, and the outlet from the apparatus 60 being selectively connected to the regeneration compartments 20a and 20b via respective control valves 62a and 62b.

As a matter of operating procedure, the plating solution may be continuously circulated from one of the reservoirs (for example, the reservoir 11a) to the plating tank 21 and back to the one reservoir 11a; and the plating solution may be continuously regenerated in the regeneration compartment 20a by the continuous addition of the reagents thereto by proper manipulation of the control valves 41, 42, 43 and 44. Of course, this regeneration of the plating solution only restores the composition thereof with respect to nickel cations, hypophosphite anions and pH, but does not restore the initial composition thereof with respect to the ions that are built-up therein, both by the plating reactions and by the additions of the reagents mentioned. In other words, as the plating solution is used in the plating operation, phosphite anions build-up therein, and likewise in the supply of make-up reagents thereto both sodium cations and sulfate anions are built-up therein (assuming that the stock solutions employed comprise nickel sulfate and sodium hypophosphite, as previously mentioned).

Accordingly, after predetermined utilization of the plating solution in the continuous plating system and continuous regeneration thereof with respect to the supply of make-up reagents thereto, it is necessary to effect a regeneration of the plating solution by the utilization of the apparatus 60 so as to bring about the removal from the plating solution of the phosphite removal from the plating solution of the phosphite anions, as well as the sodium cations and the sulfate anions. At this time, the control valve 23a is closed and the control valves 61 and 62b are opened, and operation of the apparatus 60 is initiated, as explained more fully hereinafter; whereby the plating solution from the lower portion of the secondary vacuum flash tank 15 is circulated through the apparatus 60 and thence into the regeneration compartment 20b of the reservoir 11b. At this time, the control valves 52, 53, 54 and 55 are appropriately controlled in order to cause the supply of the required make-up reagents into the regeneration compartment 20b so as substantially completely to restore the initial composition of the chemical plating solution. In order to accommodate the complete removal of the depleted plating solution from the reservoir 11a, the control valve 22a is opened to place the lower portion of the reservoir 11a into communication with the inlet of the pump 18.

In view of the foregoing, it will be understood that the depleted plating solution is circulated from the reservoir

11a through the plating tank 12 and thence into the apparatus 60 and then into the reservoir 11b. Subsequently the restored plating solution is circulated from the reservoir 11b through the plating tank 12 and thence back into the regeneration compartment 20b of the reservoir 11b, the control valves 61, 23a and 22b being operated into their closed positions and the control valves 23b and 21b being operated into their open positions at this time, whereby operation of the apparatus 60 may be arrested.

In view of the foregoing description of the mode of operation of the continuous plating system, it will be understood that as the plating solution is circulated from the reservoir 11a through the plating chamber 12, it is continuously regenerated by the addition thereto of nickel cations, hypophosphite anions and hydroxyl anions, employing the make-up equipment 30; and after a predetermined utilization thereof, it becomes necessary to regenerate it by the removal therefrom of phosphite anions, sodium cations and sulfate anions, employing the apparatus 60, followed by the addition thereto of nickel cations, hypophosphite anions and hydrogen cations, employing the make-up equipment 30. This predetermined utilization and consequent depletion of the plating solution is manifest by the build-up therein of a phosphite anion concentration within the approximate range 0.7 to 1.5 m.p.l., and is normally reached when the accumulative nickel salt addition is such that about 400% to 500% nickel cations (with respect to the initial nickel cation content of the plating solution) have been added thereto in the continuous regeneration thereof, employing the make-up equipment 30.

Considering now in greater detail the matter of the removal of the phosphite anions, together with the sodium cations and the sulfate anions, from a depleted plating bath in the apparatus 60, it is noted that any one of a number of individual treatments, described more fully hereinafter, may be employed. In the treatment, the desirable values contained in the depleted plating baths are recovered and the resulting aqueous solution is reconstituted to provide the restored plating solution. In the treatment, it is desirable first to remove from the depleted plating solution, the contained nickel cations, and this may be best done by any such conventional step which does not introduce foreign ions into the solution; i.e., electrolysis or cations exchange. Early elimination of the nickel cations is highly desirable because a variation of the pH of the solution due to reagent additions will induce a modification of the chelate stability and will result in nickel phosphite precipitation. Nickel phosphite is difficult to filter; and moreover, in order to recover the nickel, it has to be dissolved in acid and treated, which represents an additional step. Ion exchange is preferred for the nickel cation recovery over electrolysis because the latter results in an anodic oxidation of hypophosphite to phosphite. For example, a column packed with the cation exchange resin sold by Rohm and Haas under the name "Amberlite IR-120" is quite satisfactory for the present purpose; and likewise, the cation exchange resin sold by Dow under the name "Dowex 50" is entirely satisfactory.

A cation exchange resin of the type specified is ordinarily of bead-like formation and essentially comprises a stable insoluble synthetic organic polymer, active acidic functional groups chemically bonded thereto and dissociable into free mobile hydrogen cations to impart a negative charge to the polymer, and water in gel relationship with the polymer. The active acidic functional groups attached to the associated organic polymer are oriented with respect to the interfaces thereof so as to be partially or completely dissociable in the internal gel water into fixed negative ions linked to the polymer and into mobile exchangeable hydrogen cations. Typical polymers to which active acidic functional groups may be attached include: phenol-aldehyde resins, polystyrene-divinylbenzene copolymers,

and the like; and such suitable acidic functional groups include:  $-\text{SO}_3\text{H}$ ,  $-\text{COOH}$ , and the like. Normally, the water in gel relationship with the polymers should be present in the amount of at least 15% of the weight of the dry resin.

In the subsequent treatment, it is the primary object to remove a major portion of the phosphite anions, leaving, if possible, all the other constituents of the solution unchanged. Also in the treatment, it is the secondary object to remove at least a portion of the sodium cations and the sulfate anions in order to keep these ions between certain limits, i.e., at an appropriate predetermined level so as to avoid any substantial build-up thereof. In order to eliminate economically the phosphite anions, a cheap reagent has to be used, the cations of which form a phosphite compound that is less soluble than nickel phosphite, and the anions of which are identical to one of the anions already contained in the depleted solution. Moreover, this cation of the reagent mentioned cannot be a catalytic poison for the chemical nickel plating reaction (such as cadmium). Finally, the organic additives (lactic acid, etc.) contained in the solution should form soluble salts with the cation of the reagent mentioned. The last-mentioned requirement leads to a preference of Baths I and II in the continuous nickel plating process, since the salts of lactic acid and propionic acid with alkaline earth metals, and also with most heavy metals, are highly water-soluble.

In accordance with the preferred treatment of a depleted plating solution, the nickel cations are first removed therefrom by cation exchange; and to the effluent, calcium hydroxide is added in slight excess over the theoretical amount required to precipitate the phosphite anions present in the solution. The resulting solution is agitated for thirty to sixty minutes effecting substantially complete precipitation of calcium phosphite; whereupon the solution is filtered. The filter cake is then washed with cold water, whereby it consists essentially of cal-

cium phosphite, containing a small amount of calcium sulfate. The filtrate is then cooled to a relatively low temperature, about 0°-5° C., while bubbling therethrough a small amount of carbon dioxide throughout a time interval of about thirty minutes, effecting the crystallization of sodium sulfate therein and the precipitation of calcium carbonate therein. The resulting solution is then filtered, whereby the filter cake is predominantly sodium sulfate containing small amounts of calcium carbonate, sodium carbonate and sodium bicarbonate. The resulting filtrate comprises the base of a restored plating solution, since it contains substantial hypophosphite anions, as well as the organic additives (lactic acid, etc.). More particularly, to the resulting filtrate there are added nickel sulfate and sodium hypophosphite, as well as a small amount of stabilizer (such as 1-3 p.p.m. of lead ion); and then the pH of the solution is adjusted to the required value (normally about 4.6) by the addition of sulfuric acid or sodium hydroxide, if required. At this time, the reconstituted or restored plating solution is ready for use in the continuous nickel plating system.

Specifically, to the effluent mentioned the calcium hydroxide may be added in the form of an aqueous slurry and the resulting mixture is filtered to produce the corresponding filtrate.

The chemical reactions involved in this basic treatment of the depleted plating solution are as follows:



The reactions involved in the treatment of a depleted plating bath, in the manner described above, will be readily understood from the following flow sheet:

#### FLOW SHEET I

##### Depleted Bath IIB

|                             |             |     |
|-----------------------------|-------------|-----|
| $\text{Ni}^{++}$            | 0.07 - 0.08 | mpl |
| $(\text{H}_2\text{PO}_2)^-$ | 0.22 - 0.24 | mpl |
| $(\text{HPO}_3)^{--}$       | 0.75 - 0.80 | mpl |
| $\text{SO}_4^{--}$          | 0.60 - 0.70 | mpl |
| $\text{Ca}^{++}$            | none        |     |
| Lactic acid                 | 0.30        | mpl |
| Propionic acid              | 0.03        | mpl |



## Effluent

|                             |                 |
|-----------------------------|-----------------|
| $\text{Ni}^{++}$            | none            |
| $(\text{H}_2\text{PO}_2)^-$ | 0.22 - 0.24 mpl |
| $(\text{HPO}_3)^{--}$       | 0.75 - 0.80 mpl |
| $\text{SO}_4^{--}$          | 0.60 - 0.70 mpl |
| $\text{Ca}^{++}$            | none            |
| Lactic acid                 | 0.30 mpl        |
| Propionic acid              | 0.03 mpl        |

## Effluent

## Filtrate I

(above)

Add:  $\text{Ca}(\text{OH})_2$ 

|                             |                 |
|-----------------------------|-----------------|
| $\text{Ni}^{++}$            | none            |
| $(\text{H}_2\text{PO}_2)^-$ | 0.20 - 0.24 mpl |
| $(\text{HPO}_3)^{--}$       | 0.07 - 0.13 mpl |
| $\text{SO}_4^{--}$          | 0.60 - 0.70 mpl |
| $\text{Ca}^{++}$            | 0.7 - 1.6 mpl   |
| Lactic acid                 | 0.30 mpl        |
| Propionic acid              | 0.03 mpl        |

## Filter Cake I

|                             |              |           |
|-----------------------------|--------------|-----------|
| $\text{Ni}^{++}$            | none         | Dry Basis |
| $(\text{H}_2\text{PO}_2)^-$ | 0.37 - 0.44% |           |
| $(\text{HPO}_3)^{--}$       | 30.0 - 32.0% |           |
| $\text{SO}_4^{--}$          | 2.4 - 2.8%   |           |
| $\text{Ca}^{++}$            | 30.1 - 30.8% |           |
| $\text{H}_2\text{O}$        | 50.6 - 53.3% |           |

## Filtrate I

(above)

Cool to  
 $0^{\circ}$  -  $5^{\circ}$ C.; and  
 add  $\text{CO}_2$

## Filtrate II

|                               |                  |
|-------------------------------|------------------|
| $\text{Ni}^{++}$              | None             |
| $(\text{H}_2\text{PO}_2)^{-}$ | 0.19 - 0.24 mpl  |
| $(\text{HPO}_3)^{--}$         | 0.05 - 0.13 mpl  |
| $\text{SO}_4^{--}$            | 0.14 - 0.24 mpl  |
| $\text{Ca}^{++}$              | none - 0.005 mpl |
| Lactic acid                   | 0.30 mpl         |
| Propionic acid                | 0.03 mpl         |

## Filter Cake II

|                               |            |           |
|-------------------------------|------------|-----------|
| $\text{Ni}^{++}$              | none       | Dry Basis |
| $(\text{H}_2\text{PO}_2)^{-}$ | 0.1%       |           |
| $(\text{HPO}_3)^{--}$         | 0.5%       |           |
| $\text{SO}_4^{--}$            | 64.2%      |           |
| $\text{Na}^{+}$               | 28 - 33.5% |           |
| $\text{Ca}^{++}$              | 2.4%       |           |
| $\text{H}_2\text{O}$          | 64.0%      |           |

## Subject to Elution

with  $\text{H}_2\text{SO}_4$ 

## Cation Exchange Resin



Combine Filtrate II (above) with eluate (above); and then reconstitute by addition of nickel sulfate or nickel carbonate or nickel hydroxide, hypophosphorous acid, stabilizer (1-3 p.p.m.  $\text{Pb}^{++}$ ) and adjust pH to 4.6 with  $\text{NaOH}$  so as to provide the restored plating bath.

When the treatment procedure of Flow Sheet I is applied to a depleted plating bath containing succinic acid and malic acid as organic additives, such, for example, as Bath IV, approximately 10% of the succinic ions

and 10% of the malic ions are removed as the corresponding calcium salts in Filter Cake I; whereby, when Filtrate II is subsequently reconstituted, it is necessary to add corresponding amounts of succinic acid and malic acid.

In order to demonstrate the practical value of the present treatment, a depleted plating Bath IV was reconstituted to produce restored plating Bath IV in accordance with the procedure of Flow Sheet I; and then a continuous plating run was made in the continuous

plating system described utilizing this restored plating bath, with the following results:

| Cycle Number                                            | 1     | 2     | 3     | 4     |
|---------------------------------------------------------|-------|-------|-------|-------|
| Total weight gain                                       | 23.97 | 45.25 | 40.97 | 30.50 |
| Plating rate $\times 10^4$ (gm./cm. <sup>2</sup> /min.) | 3.33  | 3.14  | 3.56  | 3.53  |
| Plating rate (mils/hr.)                                 | 0.899 | 0.849 | 0.960 | 0.953 |
| Plating time (min.)                                     | 225   | 450   | 360   | 270   |
| Appearance                                              | (1)   | (1)   | (1)   | (1)   |

<sup>1</sup> Smooth and bright.

In this plating run, appropriately cleaned steel samples were nickel plated in the four cycles set forth, the nickel plating upon the samples being smooth and bright and entirely satisfactory.

5 In a modified, but less desirable, form of this treatment of the depleted plating bath, the nickel cations therein are not removed by ion exchange prior to the precipitation of the phosphite; and employing calcium hydroxide, both calcium phosphite and nickel phosphite are precipitated and removed from the resulting solution in the first filter cake. This modified procedure will be readily understood from the following flow sheet:

10

### FLOW SHEET I

#### Depleted Bath IIB

|                             |             |     |
|-----------------------------|-------------|-----|
| $\text{Ni}^{++}$            | 0.07 - 0.08 | mpl |
| $(\text{H}_2\text{PO}_2)^-$ | 0.22 - 0.24 | mpl |
| $(\text{HPO}_3)^{--}$       | 0.75 - 0.80 | mpl |
| $\text{SO}_4^{--}$          | 0.60 - 0.70 | mpl |
| $\text{Ca}^{++}$            | none        |     |
| Lactic acid                 | 0.30        | mpl |
| Propionic acid              | 0.03        | mpl |

#### Filtrate I

|                             |             |     |
|-----------------------------|-------------|-----|
| $\text{Ni}^{++}$            | none        |     |
| $(\text{H}_2\text{PO}_2)^-$ | 0.20 - 0.24 | mpl |
| $(\text{HPO}_3)^{--}$       | 0.07 - 0.13 | mpl |
| $\text{SO}_4^{--}$          | 0.60 - 0.70 | mpl |
| $\text{Ca}^{++}$            | 0.7 - 1.6   | mpl |
| Lactic acid                 | 0.30        | mpl |
| Propionic acid              | 0.03        | mpl |

Add:  
 $\text{Ca}(\text{OH})_2$

#### Filter Cake I

|                             |              |   |
|-----------------------------|--------------|---|
| $\text{Ni}^{++}$            | 2.0 - 2.5%   | } |
| $(\text{H}_2\text{PO}_2)^-$ | 0.37 - 0.44% |   |
| $(\text{HPO}_3)^{--}$       | 30.0 - 32.0% |   |
| $\text{SO}_4^{--}$          | 2.4 - 2.8%   |   |
| $\text{Ca}^{++}$            | 30.1 - 30.8% |   |
| $\text{H}_2\text{O}$        | 50.6 - 53.3% |   |

Dry Basis

## Filtrate I

(above)

Cool to 0-5°C.;  
add  $\text{CO}_2$

## Filtrate II

|                             |                   |
|-----------------------------|-------------------|
| $\text{Ni}^{++}$            | none              |
| $(\text{H}_2\text{PO}_2)^-$ | 0.19 - 0.24 mpl   |
| $(\text{HPO}_3)^{--}$       | 0.05 - 0.13 mpl   |
| $\text{SO}_4^{--}$          | 0.14 - 0.24 mpl   |
| $\text{Ca}^{++}$            | none to 0.005 mpl |
| Lactic acid                 | 0.30 mpl          |
| Propionic acid              | 0.03 mpl          |

## Filter Cake II

|                             |            |   |
|-----------------------------|------------|---|
| $\text{Ni}^{++}$            | none       | } |
| $(\text{H}_2\text{PO}_2)^-$ | 0.1%       | } |
| $(\text{HPO}_3)^{--}$       | 0.5%       | } |
| $\text{SO}_4^{--}$          | 64.2%      | } |
| $\text{Na}^+$               | 28 - 33.5% | } |
| $\text{Ca}^{++}$            | 2.4%       | } |
| $\text{H}_2\text{O}$        | 64.0%      |   |

Dry

Basis

Reconstitute Filtrate II above by the addition of nickel sulfate, etc., hypophosphorus acid, stabilizer (1-3 p.p.m.  $\text{Pb}^{++}$ ) and adjust pH to 4.6 with NaOH so as to provide the restored plating bath.

In conjunction with Flow Sheet IM, it is pointed out that the nickel contained in Filter Cake I may be recovered by dissolving the latter in sulfuric acid and then subjecting the resulting solution to ion exchange employing a cation exchange resin of the character previously specified. Thereafter, the cation exchange resin may be

subjected to elusion with sulfuric acid, the eluate containing  $\text{Ni}^{++}$  and  $\text{SO}_4^{--}$ , which eluate may be employed in conjunction with the reconstitution of Filtrate II, in the manner previously explained.

In a modified form of the treatment of the depleted plating solution, the nickel cations are first removed therefrom by cation exchange; and to the effluent, barium hydroxide is added in slight excess over the theoretical amount required to precipitate the phosphite anions pres-

ent in the solution. Specifically, to the effluent mentioned the barium hydroxide may be added in the form of an aqueous slurry and the resulting mixture is filtered to

produce the corresponding filtrate. This modified procedure will be readily understood from the following flow sheet:

FLOW SHEET II

Depleted Bath IV C

|                           |            |
|---------------------------|------------|
| $\text{NiCl}_2$           | 0.068 mpl  |
| $\text{NaH}_2\text{PO}_2$ | 0.225 mpl  |
| $\text{Na}_2\text{HPO}_3$ | 0.74 mpl   |
| Malic acid                | 0.06 mpl   |
| Lactic acid               | 0.2025 mpl |
| Succinic acid             | 0.20 mpl   |

Cation Exchange Resin



|                           |            |
|---------------------------|------------|
| $\text{Ni}^{++}$          | none       |
| $\text{NaH}_2\text{PO}_2$ | 0.225 mpl  |
| $\text{Na}_2\text{HPO}_3$ | 0.74 mpl   |
| Malic acid                | 0.06 mpl   |
| Lactic acid               | 0.2025 mpl |
| Succinic acid             | 0.20 mpl   |



Subject Filtrate II above to the cooling and  $\text{CO}_2$  contact steps disclosed in Flow Sheet I in order to precipitate  $\text{Na}_2\text{SO}_4$ , etc., and filter to produce Filter Cake III con-

sisting fundamentally of  $\text{Na}_2\text{SO}_4$  and Filtrate III corresponding to Filtrate II above (after the removal of 75  $\text{Na}_2\text{SO}_4$ ).

23

Then reconstitute Filtrate III mentioned above by the addition thereto of nickel chloride, malic acid, succinic acid, and adjust the pH to 4.6 with NaOH so as to provide the restored plating bath.

In conjunction with Flow Sheet II, it will be observed that substantially all barium ions in Filtrate I are removed therefrom by the addition of sulfuric acid bringing about the precipitation of barium sulfate.

Just as the treatment of Flow Sheet I was modified to produce Flow Sheet IM, as explained above, Flow Sheet II may be modified to produce a corresponding Flow Sheet IIM. In this modified treatment of the depleted plating bath, the nickel cations therein are not removed by the ion exchange prior to the precipitation of the phosphite, and when the barium hydroxide is added to the depleted plating bath, both barium phosphite and

24

nickel phosphite are precipitated and removed from the resulting solution in the first filter cake. This modified procedure is not set forth in further detail in the interest of brevity.

5 In another modified form of the treatment of the depleted plating solution, the nickel cations are first removed therefrom by cation exchange; and to the effluent, magnesium carbonate is added in slight excess over the theoretical amount required to precipitate the phosphite anions present in the solution. Specifically, to the effluent mentioned the magnesium carbonate may be added in the form of a powder or an aqueous slurry and the resulting mixture is filtered to produce the corresponding filtrate. This modified procedure will be readily understood from the following flow sheet:

### FLOW SHEET III

#### Depleted Bath IV B

|                           |      |     |
|---------------------------|------|-----|
| $\text{Ni}^{++}$          | 0.07 | mpl |
| $\text{NaH}_2\text{PO}_2$ | 0.20 | mpl |
| $\text{Na}_2\text{HPO}_3$ | 0.86 | mpl |
| Malic acid                | 0.06 | mpl |
| Lactic acid               | 0.20 | mpl |
| Succinic acid             | 0.20 | mpl |

#### Cation Exchange Resin



#### Effluent

|                           |          |
|---------------------------|----------|
| $\text{Ni}^{++}$          | none     |
| $\text{NaH}_2\text{PO}_2$ | 0.20 mpl |
| $\text{Na}_2\text{HPO}_3$ | 0.86 mpl |
| Malic acid                | 0.06 mpl |
| Lactic acid               | 0.20 mpl |
| Succinic acid             | 0.20 mpl |

## Effluent



## Filtrate I

|                                  |          |
|----------------------------------|----------|
| NaH <sub>2</sub> PO <sub>2</sub> | 0.20 mpl |
| Na <sub>2</sub> HPO <sub>3</sub> | 0.15 mpl |
| Malic acid                       | 0.03 mpl |
| Lactic acid                      | 0.20 mpl |
| Succinic acid                    | 0.20 mpl |
| Mg <sup>++</sup>                 | 0.1 mpl  |

## Filter Cake I

|                                |       |
|--------------------------------|-------|
| HPO <sub>3</sub> <sup>--</sup> | 44.1% |
| Mg <sup>++</sup>               | 8.4%  |
| H <sub>2</sub> O               | 43.3% |
| Malic acid                     |       |

Subject Filtrate I above to the cooling and CO<sub>2</sub> contact steps disclosed in Flow Sheet I in order to precipitate Na<sub>2</sub>SO<sub>4</sub>, etc.; and filter to produce Filter Cake II consisting fundamentally of Na<sub>2</sub>SO<sub>4</sub> and Filtrate II corresponding to Filtrate I above (after the removal of Na<sub>2</sub>SO<sub>4</sub>).

Then reconstitute Filtrate II mentioned above by the addition thereto of nickel sulfate, sodium hypophosphite, malic acid and stabilizer (1-3 p.p.m. Pb<sup>++</sup>), and adjust pH to 4.6 with NaOH so as to provide the restored plating bath.

In conjunction with Flow Sheet III, it is noted that small amounts of magnesium cations are introduced into Filtrate I that are carried into the ultimately reconstituted or restored plating bath. Further, it will be appreciated that in addition to precipitating the phosphite anions as magnesium phosphite, by metastatic exchange, the magnesium carbonate also removes phosphite and some hypophosphite and sulfate anions by adsorption in Filter Cake I, as magnesium carbonate is an anion adsorption material with respect to these anions. However, the magnesium carbonate carries into Filter Cake I by adsorption no substantial proportion of malic, lactic or succinic anions, or other weakly acidic bath constituents. Moreover, the reconstitution of Filtrate II may involve the addition of nickel carbonate or nickel hydroxide and the addition of hypophosphorous acid, as explained in connection with Flow Sheet I above. Of course, it will be understood, that the utilization of nickel carbonate and nickel hydroxide in the reconstitution of Filtrate II also increases the pH thereof, whereby it may be necessary to add an acid (H<sub>2</sub>SO<sub>4</sub>) to Filtrate II to obtain the desired pH of about 4.6 of the reconstituted plating bath.

Just as the treatment of Flow Sheet I was modified to produce Flow Sheet IM, as explained above, Flow Sheet III may be modified to produce a corresponding Flow Sheet IIM. In this modified treatment of the depleted plating bath, the nickel cations therein are not removed by

ion exchange prior to the precipitation of the phosphites, and when the magnesium carbonate is added to the depleted plating bath, both magnesium phosphite and nickel phosphite are precipitated and removed from the resulting solution in the first filter cake. This modified procedure is not set forth in further detail in the interest of brevity.

In the foregoing treatment procedures, the depleted plating baths were restored substantially to the initial compositions thereof by the complete removal of substantially all of the phosphite and other foreign ions, together with the additions of the nickel cations and the hypophosphite anions; however, substantial advantages and economies may be achieved in the continuous process of chemical nickel process by utilizing more simplified procedures that do not necessarily restore the depleted plating bath to its initial composition, but that do remove phosphite anions therefrom and supply nickel cations and hypophosphite anions thereto.

For example, a depleted plating bath of any one of the types previously mentioned may be restored to its approximate initial composition in a simple and ready manner by adding thereto a suitable quantity of nickel hypophosphite, nickel sulfate, nickel carbonate, nickel hydroxide, or other nickel salt, and a suitable quantity of nickel hypophosphite, sodium hypophosphite, hypophosphorous acid, or other hypophosphite, followed by contacting the resulting solution with freshly precipitated or active aluminum hydroxide. Specifically, the freshly precipitated Al(OH)<sub>3</sub> may be added and stirred into the solution, while heating the same, for about one hour. Thereafter, the resulting slurry is filtered and the pH of the filtrate is adjusted with a suitable acid to produce a restored plating bath. This arrangement is very advantageous as the freshly precipitated or active Al(OH)<sub>3</sub> comprises an anion adsorption material for phosphite and sulfate anions, as well as to some extent for hypophosphite anions, but the required amount of hypophosphite anions may be added to compensate for this effect; whereby the undesirable phosphite and sulfate an-

ions are removed from the depleted plating bath. This arrangement is very simple, introduces no foreign ions into the resulting restored plating bath, and can be carried out with substantially no chemical controls, after the initial procedure is established. Moreover, the arrangement meets all of the fundamental requirements of regeneration as it supplies needed nickel cations and hypophosphite anions and removes undesirable phosphite and sulfate anions.

In order to demonstrate this procedure, a plating bath was initially composed comprising:

|                                            |        |        |
|--------------------------------------------|--------|--------|
| NiSO <sub>4</sub> -----                    | m.p.l. | 0.1125 |
| NaH <sub>2</sub> PO <sub>2</sub> -----     | m.p.l. | 0.225  |
| NH <sub>2</sub> CH <sub>2</sub> COOH ----- | m.p.l. | 0.180  |
| NaOH -----                                 | m.p.l. | 0.120  |
| pH -----                                   |        | 6.48   |

With this plating solution, properly cleaned steel samples were plated in a plating chamber having a volume of about 300 cc. employing 2000 cc. of the plating solution, the plating solution being continuously flowed through the plating chamber at a rate of about 50 cc. per minute and the temperature thereof in the plating chamber being maintained at about 96° to 97° C. In this plating test 0.6807 gm. of bright smooth plating was produced upon the steel samples, whereby the plating rate was  $4.34 \times 10^{-4}$  gm./cm.<sup>2</sup>/min. The time of the test was 40 minutes; the solution remained clear in the test; and the pH thereof was decreased from 6.48 to 6.01.

Thereafter the plating solution was partially regenerated by adding thereto 4.25 gms. of Ni(H<sub>2</sub>PO<sub>2</sub>)<sub>2</sub>; and to the solution a quantity of freshly precipitated Al(OH)<sub>3</sub> was added and stirred therein for a time interval of one hour. The resulting slurry was then filtered and the pH of the filtrate was 6.5.

The filtrate mentioned was utilized directly as a regenerated plating solution and therewith properly cleaned steel samples were again plated in the plating chamber with 2060 cc. of the solution, the plating solution being continuously flowed through the plating chamber at a rate of about 53 cc. per minute, and the temperature thereof in the plating chamber being maintained at about 97° C. In this plating test 0.7674 gm. of bright smooth plating was produced upon the steel samples, whereby the plating rate was  $5.00 \times 10^{-4}$  gm./cm.<sup>2</sup>/min. The time of the test was 39 minutes; the solution remained clear in the test; and the pH thereof was decreased from 6.50 to 6.13.

Thereafter the plating solution was again partially regenerated by adding thereto 3.35 gms. of Ni(H<sub>2</sub>PO<sub>2</sub>)<sub>2</sub>; and to the solution a quantity of freshly precipitated Al(OH)<sub>3</sub> was added and stirred therein for a time interval of one hour. The resulting slurry was then filtered and the pH of the filtrate was adjusted to 6.42.

The filtrate mentioned was utilized directly as a regenerated plating solution and therewith properly cleaned steel samples were again plated in the plating chamber with 2000 cc. of the solution, the plating solution being continuously flowed through the plating chamber at a rate of about 57 cc. per minute and the temperature thereof in the plating chamber being maintained at about 96° C. In this plating test 0.7767 gm. of bright smooth plating was produced upon the steel samples, whereby the plating rate was  $5.35 \times 10^{-4}$  gm./cm.<sup>2</sup>/min. The time of the test was 35 minutes; the solution remained clear in the test; and the pH thereof was decreased from 6.42 to 6.15.

Thereafter the plating solution was again partially regenerated by adding thereto 3.64 gms. of Ni(H<sub>2</sub>PO<sub>2</sub>)<sub>2</sub>; and to the solution a quantity of freshly precipitated Al(OH)<sub>3</sub> was added and stirred therein for a time interval of one hour. The resulting slurry was then filtered and the pH of the filtrate was adjusted to 6.39.

The filtrate mentioned was utilized directly as a regenerated plating solution and therewith properly cleaned steel samples were again plated in the plating chamber with 2000 cc. of the solution, the plating solution being continuously flowed through the plating chamber at a rate

of about 57 cc. per minute, and the temperature thereof in the plating chamber being maintained at about 97° C. In this plating test 0.7386 gm. of plating was produced upon the steel samples, whereby the plating rate was  $5.37 \times 10^{-4}$  gm./cm.<sup>2</sup>/min. The time of the test was 35 minutes; the solution remained clear in the test; and the pH thereof was decreased somewhat below 6.39.

Another approximate regeneration procedure was devised that is predicated upon regeneration with nickel hydroxide and hypophosphorous acid for the purpose of supplying the required nickel cations and hypophosphite anions, and upon utilization of the adsorption characteristic of the nickel hydroxide for the removal of undesirable phosphite anions.

In accordance with this procedure, an initial aqueous slurry was prepared having the composition:

|                                                             |        |       |
|-------------------------------------------------------------|--------|-------|
| Ni(OH) <sub>2</sub> -----                                   | mole   | 0.45  |
| H <sub>3</sub> PO <sub>3</sub> -----                        | gms    | 10    |
| NaCl -----                                                  | gms    | 21.1  |
| H <sub>3</sub> PO <sub>2</sub> -----                        | gms    | 79.2  |
| Malonic acid -----                                          | gms    | 18.75 |
| "Dialite" (filter aid) -----                                | gms    | 40.0  |
| Tap water -----                                             | liters | 2     |
| The pH of the wet Ni(OH) <sub>2</sub> as prepared was ----- |        | 8.23  |

The slurry was thoroughly agitated until the pH thereof became constant at about 6.30 after 7 hours of agitation. Then the slurry was filtered and 3200 cc. of filtrate was obtained having a pH of 6.35.

The filtrate was employed as a plating solution and therewith properly cleaned steel samples were plated in a plating chamber having a volume of about 300 cc. employing 3200 cc. of the plating solution, the plating solution being continuously flowed through the plating chamber at a rate of about 55 cc. per minute, and the temperature thereof in the plating chamber being maintained at about 98° C. In this plating test 1.2273 gms. of bright smooth plating was produced upon the steel samples, whereby the plating rate was  $2.69 \times 10^{-4}$  gm./cm.<sup>2</sup>/min. The time of the test was 58 minutes; the solution remained clear in the test; and the pH thereof was decreased from 6.35 to 4.33.

Thereafter the plating solution was partially regenerated by adding the same back to the filter cake that was produced by the filtering of the initial slurry, the filter cake mentioned having been ground into finely divided form, whereby a new slurry was produced after an addition of malonic acid and water, that had the following composition:

|                                      |        |        |
|--------------------------------------|--------|--------|
| Ni(OH) <sub>2</sub> -----            | m.p.l. | 0.3    |
| NaCl -----                           | m.p.l. | 0.24   |
| H <sub>3</sub> PO <sub>2</sub> ----- | m.p.l. | 0.227  |
| H <sub>3</sub> PO <sub>3</sub> ----- | m.p.l. | 0.0122 |
| Malonic acid -----                   | m.p.l. | 0.12   |
| Filter aid (total) -----             | gms    | 40     |
| Volume of slurry -----               | liters | 4      |

This new slurry was thoroughly agitated until the pH thereof came to equilibrium at 6.19 after about 7 hours, whereupon the same was filtered, the filtrate had a volume of 3400 cc. and a pH of 6.03. The pH of the filtrate was then adjusted to 5.42 with acid, and 3200 cc. thereof was employed as a plating bath, and therewith properly cleaned steel samples were plated in the plating chamber, the plating solution being continuously flowed through the plating chamber at a rate of about 61.5 cc. per minute, and the temperature thereof in the plating chamber being maintained at about 98° C. In this plating test 0.7293 gms. of bright smooth plating was produced upon the steel samples, whereby the plating rate was  $1.78 \times 10^{-4}$  gm./cm.<sup>2</sup>/min. The time of the test was 52 minutes; the solution remained clear in the test; and the pH thereof was decreased from 5.42 to 4.52.

In view of the foregoing, it will be understood that in the continuous chemical nickel plating process, the ef-

fective or useful life of the initial plating solution may be greatly extended by the regeneration thereof, including the removal of the deleterious phosphite anions therefrom; and the treatment of Flow Sheet I is especially recommended in view of the circumstance that it is the most advantageous of all of the treatments disclosed with respect to the removal from the plating solution of phosphite anions, sodium cations and sulfate anions, without the introduction thereinto of foreign ions, whereby the plating solution may be restored any number of times after a corresponding number of intervening depletions thereof.

In the foregoing description, periodic or intermittent regeneration of the plating solution, with respect to the removal of phosphite anions, sodium cations and sulfate anions, in the continuous plating system was explained; however, it will be understood that this regeneration of the plating solution in the system may be continuous. This may be accomplished in a ready manner by opening the control valves 61 and 62a (utilizing the reservoir 11a) so that the apparatus 60 is arranged in by-passing relation with respect to the direct return of the plating solution to the regeneration compartment 20a. The control valve 23a also being open at this time. Thus in this arrangement, two portions of the plating solution from the lower portion of the secondary vacuum flash tank 15 respectively flow directly into the regeneration compartment 20a via the control valve 23a and indirectly into the regeneration compartment 20a via the control valve 61 and the apparatus 60. By treatment of the portion of the plating solution passing through the apparatus 60, in the manner previously explained, the required removal of phosphite anions, sodium cations and sulfate anions may be accomplished upon a continuous basis so as to prevent excessive depletion thereof in the continuous plating operation.

Accordingly, it will be understood that there has been provided a continuous chemical nickel plating process that is highly suitable for use on an industrial scale, that involves regeneration of the plating bath, as it becomes depleted with use, in a simple manner, thereby rendering the plating bath of exceedingly long life and contributing to overall efficiency of the continuous chemical nickel plating process.

While there has been described what is at present considered to be the preferred embodiment of the invention, it will be understood that various modifications may be made therein, and it is intended to cover in the appended claims all such modifications as fall within the true spirit and scope of the invention.

What is claimed is:

1. In the continuous process of chemically plating with nickel a body of catalytic material that involves providing an aqueous plating solution of the nickel cation-hypophosphite anion type and having an initial composition including a pH in a first given range and a nickel cation concentration in a second given range and a hypophosphite anion concentration in a third given range, holding said solution in a plating chamber at a plating temperature disposed below the boiling point thereof but well above room temperature, immersing said body in said solution in said plating chamber to effect nickel plating on the surface thereof, and withdrawing said body from the portion of said solution in said plating chamber after a time interval corresponding to the thickness of the nickel plating on the surface of said body that is desired, said nickel plating of said body resulting from the reduction of nickel cations to metallic nickel with the corresponding oxidation of hypophosphite anions to phosphite anions, whereby during said time interval both nickel cations and hypophosphite anions are depleted and both hydrogen cations and phosphite anions are produced in said solution in said plating chamber, with the result that said solution in said plating chamber tends to depart substantially from said initial composition; the improve-

ment comprising withdrawing during said time interval a part of said solution from said plating chamber, treating during said time interval the withdrawn part of said solution to restore the same substantially to said initial composition, and returning during said time interval said restored part of said solution into said plating chamber, said treatment of the withdrawn part of said solution including reacting the same with an alkaline earth hydroxide to precipitate a corresponding alkaline earth phosphite therein, separating the precipitated alkaline earth phosphite from the resulting solution, and adding to the resulting solution sufficient pH control ions to restore the pH thereof into said first range and sufficient nickel cations to restore the concentration thereof into said second range and sufficient hypophosphite anions to restore the concentration thereof into said third range.

2. In the continuous process of chemically plating with nickel a body of catalytic material that involves providing an aqueous plating solution of nickel sulfate and sodium hypophosphite and having an initial composition including a pH in a first given range and a nickel cation concentration in a second given range and a hypophosphite anion concentration in a third given range, holding said solution in a plating chamber at a plating temperature disposed below the boiling point thereof but well above room temperature, immersing said body in said solution in said plating chamber to effect nickel plating on the surface thereof, and withdrawing said body from said solution in said plating chamber after a time interval corresponding to the thickness of the nickel plating on the surface of said body that is desired, said nickel plating of said body resulting from the reduction of nickel cations to metallic nickel with the corresponding oxidation of hypophosphite anions to phosphite anions, whereby during said time interval both nickel cations and hypophosphite anions are depleted and both hydrogen cations and phosphite anions are produced in said solution in said plating chamber, with the result that said solution in said plating chamber tends to depart substantially from said initial composition; the improvement comprising withdrawing during said time interval a part of said solution from said plating chamber, treating during said time interval the withdrawn part of said solution to restore the same substantially to said initial composition, and returning during said time interval said restored part of said solution into said plating chamber, said treatment of the withdrawn part of said solution including reacting the same with an alkaline earth hydroxide to precipitate a corresponding alkaline earth phosphite therein, separating the precipitated alkaline earth phosphite from the resulting solution, cooling the resulting solution to crystallize out sodium sulfate therein, separating the crystallized sodium sulfate from the resulting solution, and adding to the resulting solution sufficient pH control ions to restore the pH thereof into said first range and sufficient nickel sulfate to restore the nickel cation concentration thereof into said second range and sufficient sodium hypophosphite to restore the hypophosphite anion concentration thereof into said third range.

3. The process of regenerating a depleted aqueous chemical nickel plating solution containing substantial nickel cations and substantial hypophosphite anions and considerable phosphite anions and a given organic additive to produce a restored aqueous chemical nickel plating solution containing a predetermined nickel cation concentration and a predetermined hypophosphite anion concentration and only some phosphite anions and substantially said given organic additive and having a given pH, which comprises contacting a mass of cation exchange material with said solution to remove nickel cations therefrom, reacting the resulting solution with an alkaline earth hydroxide to precipitate a corresponding alkaline earth phosphite therein, separating the precipitated alkaline earth phosphite from the resulting solution, whereby the resulting solution contains only some nickel

cations and some phosphite anions and considerable hypophosphite anions and substantially said given organic additive, and adding to the resulting solution sufficient nickel cations to obtain said predetermined nickel cation concentration therein and sufficient hypophosphite anions to obtain said predetermined hypophosphite anion concentration therein and sufficient pH control ions to obtain said given pH thereof.

4. The process of regenerating a depleted aqueous chemical nickel plating solution containing substantial nickel cations and substantial hypophosphite anions and considerable sodium cations and considerable phosphite anions and considerable sulfate anions to produce a restored aqueous chemical nickel plating solution containing a predetermined nickel cation concentration and a predetermined hypophosphite anion concentration and only some sodium cations and only some phosphite anions and only some sulfate anions and having a given pH, which comprises contacting a mass of cation exchange material with said solution to remove nickel cations therefrom, reacting the resulting solution with an alkaline earth hydroxide to precipitate a corresponding alkaline earth phosphite therein, separating the precipitated alkaline earth phosphite from the resulting solution, cooling the resulting solution to crystallize out sodium sulfate therein, separating the crystallized sodium sulfate from the resulting solution, whereby the resulting solution contains only some nickel cations and some sodium cations and some phosphite anions and some sulfate anions and considerable hypophosphite anions, and adding to the resulting solution sufficient nickel sulfate to obtain said predetermined nickel cation concentration therein and sufficient sodium hypophosphite to obtain said predetermined hypophosphite anion concentration therein and sufficient pH control ions to obtain said given pH thereof.

5. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises contacting a mass of cation exchange material with said solution to remove nickel cations therefrom, reacting the resulting solution with an alkaline earth hydroxide to precipitate a corresponding alkaline earth phosphite therein, separating the precipitated alkaline earth phosphite from the resulting solution, and adding to the resulting solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

6. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises contacting a mass of cation exchange material with said solution to remove nickel cations therefrom, reacting the resulting solution with calcium hydroxide to precipitate calcium phosphite therein, separating the precipitated calcium phosphite from the resulting solution, and adding to the resulting solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

7. The process of regenerating a depleted aqueous

chemical nickel plating solution containing substantial nickel cations and substantial hypophosphite anions and considerable sodium cations and considerable phosphite anions and considerable sulfate anions to produce a restored aqueous chemical nickel plating solution containing a predetermined nickel cation concentration and a predetermined hypophosphite anion concentration and only some sodium cations and only some phosphite anions and only some sulfate anions and having a given pH, which comprises contacting a mass of cation exchange material with said solution to remove nickel cations therefrom, reacting the resulting solution with an alkaline earth hydroxide to precipitate a corresponding alkaline earth phosphite therein, separating the precipitated alkaline earth phosphite from the resulting solution, cooling the resulting solution to a temperature within the approximate range 0 to 5° C. to crystallize out sodium sulfate therein, separating the crystallized sodium sulfate from the resulting solution, and adding to the resulting solution sufficient nickel sulfate to obtain said predetermined nickel cation concentration therein and sufficient sodium hypophosphite to obtain said predetermined hypophosphite anion concentration therein and sufficient pH control ions to obtain said given pH thereof.

8. The process of regenerating a depleted aqueous chemical nickel plating solution containing substantial nickel cations and substantial hypophosphite anions and considerable sodium cations and considerable phosphite anions and considerable sulfate anions to produce a restored aqueous chemical nickel plating solution containing a predetermined nickel cation concentration and a predetermined hypophosphite anion concentration and only some sodium cations and only some phosphite anions and only some sulfate anions and having a given pH, which comprises contacting a mass of cation exchange material with said solution to remove nickel cations therefrom, reacting the resulting solution with calcium hydroxide to precipitate calcium phosphite therein, separating the precipitated calcium phosphite from the resulting solution, cooling the resulting solution to a temperature within the approximate range 0 to 5° C. to crystallize out sodium sulfate therein and reacting the same with carbon dioxide to precipitate calcium carbonate therein, removing the crystallized sodium sulfate and the precipitated calcium carbonate from the resulting solution, and adding to the resulting solution sufficient nickel sulfate to obtain said predetermined nickel cation concentration therein and sufficient sodium hypophosphite to obtain said predetermined hypophosphite anion concentration therein and sufficient pH control ions to obtain said given pH thereof.

9. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises contacting a mass of cation exchange resin with said depleted solution in order to effect the removal of nickel cations therefrom, reacting the resulting effluent with an alkaline earth hydroxide to precipitate a corresponding alkaline earth phosphite therein, separating the precipitated alkaline earth phosphite from the reacted solution, subjecting said mass of cation exchange resin to elution with an acid, whereby the eluate contains nickel cations removed from said mass of ion exchange resin, combining the reacted solution and the eluate, and adding to the combined solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

10. The process of treating a depleted chemical nickel plating solution of the nickel cation-hypophosphite anion type also containing phosphite anions, said process comprising reacting said solution with an alkaline earth hydroxide to precipitate a corresponding alkaline earth phosphite therein, separating the precipitated alkaline earth phosphite from the resulting solution, and adding to the resulting solution nickel cations and hypophosphite anions to produce a restored chemical nickel plating solution containing predetermined nickel cations and predetermined hypophosphite anions.

11. The process set forth in claim 10, wherein said alkaline earth hydroxide is selected from the class consisting of barium hydroxide and calcium hydroxide.

12. The process of regenerating a depleted chemical nickel plating solution of the nickel cation-hypophosphite anion type also containing phosphite anions and sodium cations and sulfate anions, said process comprising reacting said solution with an alkaline earth hydroxide to precipitate a corresponding alkaline earth phosphite therein, separating the precipitated alkaline earth phosphite from the resulting solution, cooling the resulting solution to a temperature in the approximate range 0° to 5° C. to crystallize out sodium sulfate therein, separating the crystallized sodium sulfate from the resulting solution, and then adding to the resulting solution both nickel sulfate and sodium hypophosphite to produce a restored chemical nickel plating solution containing predetermined nickel cations and predetermined hypophosphite anions.

13. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises reacting said depleted solution with an alkaline earth hydroxide to precipitate both nickel phosphite and a corresponding alkaline earth phosphite therein, separating the precipitated nickel phosphite and alkaline earth phosphite from the resulting solution, and adding to the resulting solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

14. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises reacting said depleted solution with calcium hydroxide to precipitate both nickel phosphite and calcium phosphite therein, separating the precipitated nickel phosphite and calcium phosphite from the resulting solution, and adding to the resulting solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

15. The process of regenerating a depleted aqueous chemical nickel plating solution containing substantial nickel cations and substantial hypophosphite anions and considerable sodium cations and considerable phosphite anions and considerable sulfate anions to produce a restored aqueous chemical nickel plating solution containing a predetermined nickel cation concentration and a predetermined hypophosphite anion concentration and only

5 some sodium cations and only some phosphite anions and only some sulfate anions and having a given pH, which comprises reacting said depleted solution with an alkaline earth hydroxide to precipitate both nickel phosphite and a corresponding alkaline earth phosphite therein, separating the precipitated nickel phosphite and alkaline earth phosphite from the resulting solution, cooling the resulting solution to a temperature within the approximate range 0 to 5° C. to crystallize out sodium sulfate therein, separating the crystallized sodium sulfate from the resulting solution, and adding to the resulting solution sufficient nickel sulfate to obtain said predetermined nickel cation concentration therein and sufficient sodium hypophosphite to obtain said predetermined hypophosphite anion concentration therein and sufficient pH control ions to obtain given pH thereof.

16. The process of regenerating a depleted aqueous chemical nickel plating solution containing substantial nickel cations and substantial hypophosphite anions and considerable sodium cations and considerable phosphite anions and considerable sulfate anions to produce a restored aqueous chemical nickel plating solution containing a predetermined nickel cation concentration and a predetermined hypophosphite anion concentration and only some sodium cations and only some phosphite anions and only some sulfate anions and having a given pH, which comprises reacting said depleted solution with calcium hydroxide to precipitate both nickel phosphite and calcium phosphite therein, separating the precipitated nickel phosphite and calcium phosphite from the resulting solution, cooling the resulting solution to a temperature within the approximate range 0 to 5° C. to crystallize out sodium sulfate therein and reacting the same with carbon dioxide to precipitate calcium carbonate therein, separating the sodium sulfate and calcium carbonate from the resulting solution, and adding to the resulting solution sufficient nickel sulfate to obtain said predetermined nickel cation concentration therein and sufficient sodium hypophosphite to obtain said predetermined hypophosphite anion concentration therein and sufficient pH control ions to obtain said given pH thereof.

17. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises 45 contacting a mass of cation exchange material with said solution to remove nickel cations therefrom, reacting the resulting solution with barium hydroxide to precipitate barium phosphite therein, separating the precipitated barium phosphite from the resulting solution, reacting the resulting solution with sulfuric acid to precipitate barium sulfate therein, separating the precipitated barium sulfate from the resulting solution, and adding to the resulting solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

18. The process of regenerating a depleted aqueous chemical nickel plating solution containing substantial nickel cations and substantial hypophosphite anions and considerable phosphite anions to produce a restored aqueous chemical nickel plating solution containing a predetermined nickel cation concentration and a predetermined hypophosphite anion concentration and only some phosphite anions and having a given pH, which comprises 65 contacting a mass of cation exchange material with said solution to remove nickel cations therefrom, contacting the resulting solution with magnesium carbonate to remove phosphite anions therefrom, separating the resulting magnesium phosphite from the resulting solution, and

adding to the resulting solution sufficient soluble nickel salt to obtain said predetermined nickel cation concentration therein and sufficient soluble hypophosphite to obtain said predetermined hypophosphite anion concentration therein and sufficient pH control ions to obtain said given pH thereof.

19. In a chemical reduction nickel plating process utilizing an aqueous solution containing nickel cations and a hypophosphite reducing agent, the improvement which consists of dissolving in said solution a nickel compound, thereby to prevent during the process undesirable depletion of nickel cations in said solution, reacting said solution with an alkaline earth hydroxide to precipitate a corresponding alkaline earth phosphite therein, and separating said precipitated alkaline earth phosphite from said solution, thereby to prevent during the process undesirable build-up of phosphite anions in said solution.

20. The process set forth in claim 19, wherein said nickel compound is selected from the group consisting of nickel hydroxide and nickel carbonate.

21. In a chemical reduction nickel plating process utilizing a plating bath comprising an aqueous solution containing a water-soluble nickel salt and a hypophosphite reducing agent, the improvement which consists of replenishing the hypophosphite in said bath by addition of hypophosphorous acid, and treating said bath with an anion adsorption material to remove phosphite ions produced by said process, wherein said anion adsorption material comprises aluminum hydroxide.

22. A method of treating chemical reduction plating solutions, said method comprising passing said solution through an anion adsorption material capable of adsorbing phosphite ions from said solution, wherein said anion adsorption material comprises aluminum hydroxide, and adding a hypophosphite reducing agent to said solution.

23. The process of treating a depleted chemical nickel

5 plating solution of the nickel cation-hypophosphite anion type also containing phosphite anions, said process comprising contacting a mass of anion adsorption material with said solution to remove phosphite anions therefrom, wherein said anion adsorption material comprises aluminum hydroxide, and adding to the resulting solution nickel cations and hypophosphite anions.

## References Cited

## UNITED STATES PATENTS

|           |         |            |       |            |
|-----------|---------|------------|-------|------------|
| 2,532,283 | 12/1950 | Brenner    | ----- | 117—130    |
| 2,658,839 | 11/1953 | Talmey     | ----- | 117—102    |
| 2,658,842 | 11/1953 | Gutzeit    | ----- | 117—130    |
| 2,717,218 | 9/1955  | Talmey     | ----- | 117—102    |
| 2,726,968 | 12/1955 | Spaulding  | ----- | 117—102 XR |
| 2,726,969 | 12/1955 | Spaulding  | ----- | 117—102    |
| 2,871,142 | 1/1959  | Hays.      |       |            |
| 2,886,451 | 6/1959  | Budinikas. |       |            |
| 2,886,452 | 6/1959  | Duvall.    |       |            |

10  
15  
20

25

## OTHER REFERENCES

Costa, Industrial and Engineering Chemistry, vol. 42, No. 2, February 1950 (pp. 308 to 311 relied on), copy available in Class 210—24.1.

Kunin, Ion Exchange Resins, 1950, John Wiley & Sons, Inc., New York, pp. 135 to 139 relied on, copy available in Div. 50.

Paulson, Plating, vol. 40, No. 9, September 1953, pp. 1005 to 1009 relied on, copy available in Class 210—24.1.

ALEXANDER H. BRODMERKEL, *Primary Examiner.*

RICHARD D. NEVIUS, *Examiner.*

35 R. BLANKE, R. S. KENDALL, D. J. ARNOLD,  
*Assistant Examiners.*

30